# EUROPEAN PATENT SPECIFICATION

(11) **EP 2 054 539 B1**
(45) Date of publication and mention of the grant of the patent: **30.05.2012**
(21) Application number: 07786477.5
(22) Date of filing: 31.07.2007
(51) Int. Cl.: C25D 3/06, C25D 21/12, C25D 17/00

(54) **METHOD FOR DEPOSITION OF CHROMIUM LAYERS AS HARD- CHROME PLATING, ELECTROPLATING BATH AND HARD- CHROME SURFACES**
VERFAHREN ZUR ABSCHEIDUNG VON CHROMSCHICHTEN ALS HARTVERCHROMUNG, GALVANISIERUNGSBAD SOWIE HARTVERCHROMTE OBERFLÄCHEN
PROCÉDÉ DE DÉPÔT DE COUCHES DE CHROME SOUS FORME DE PLACAGE AU CHROME DUR, BAIN GALVANOPLASTIQUE ET SURFACES À BASE DE CHROME DUR

(30) Priority: 01.08.2006 DE 102006035871
(43) Date of publication of application: 06.05.2009
(73) Proprietor: Fraunhofer-Gesellschaft zur Förderung der angewandten Forschung e.V., 80686 München (DE)
(72) Inventor: BOHNET, Jens, 72290 Lossburg (DE); METZNER, Martin, 74417 Gschwend (DE); KRASSNITZER, Herwig, A-9330 Althofen (AT); SCHERMANZ, Karl, A-9314 Launsdorf (AT)
(74) Representative: Pfenning, Meinig & Partner GbR
(86) International application number: PCT/EP2007/006783
(87) International publication number: WO 2008/014987

(56) References cited:
- GB-A- 2 290 553
- JP-A- 61 023 783
- JP-A- 61 026 797
- JP-A- 61 288 100
- US-A1- 2005 189 231

## Description

### FIELD OF THE INVENTION

The invention relates to a method for deposition of chromium layers as hard-chrome plating for protection against wear or corrosion and/or for decorative purposes and also an electroplating bath with which chromium layers of this type can be deposited. The invention also relates to hard-chrome surfaces produced accordingly.

### DESCRIPTION OF PRIOR ART

In the case of commercial methods which have become known to date from prior art for producing thick chromium coatings, electrolytes in which the chromium to be deposited is present in a hexavalent form are used virtually exclusively.

Efforts have been made since the beginning of electrolytic chromium deposition to replace the toxic chromium(VI) electrolytes by chromium(III) electrolytes. The attempt to replace the chromium(VI) compounds by chromium(III) compounds starts from the fact that chromium(VI) compounds which pass into the body can lead to serious health problems. In addition to health and environmentally endangering aspects, also high costs arise for disposal of chromium(VI)-polluted waste waters.

In general, a distinction must be made between the deposition of decorative, thin (< 3 µm) chromium layers for glossy chroming, obtaining metallic chromium from chromium(III)-containing solutions and the deposition of thick (> 5 µm) chromium layers as wear- and corrosion protection layers.

There are already numerous methods and patents for decorative chrome plating which deal with this topic. These methods produce a thin high-gloss chromium layer. For layer thicknesses above 5 µm, these methods are however only suitable in a restricted manner.

In the last few years, there have been numerous attempts to replace industrial chroming from chromium(VI)-containing processes by processes based on chromium(III).

An electroplating bath for the deposition of chromium layers is known from GB 1 602 404 which is based on chromium(III). In this case, the separation between catholyte and anolyte is effected by means of a cation exchanger membrane. Anions for reducing the deposition voltage are added here to the catholyte, as a result of which an increase in the voltage during the electroplating can be avoided.

GB 2 290 553 A describes a chromium plating method using a plating bath comprising trivalent chromium and an electrode, wherein the electrode is an anode comprising an electrode substrate coated with an electrode catalyst comprising iridium oxide.

JP 61-026797 A describes a chromium alloy plating method of metals, such as Cr and Ni, Fe, by using an electrolytic cell in which cathode and anode chambers are divided with an ion exchanger film.

JP 61-23783 A describes a method for plating chromium using an electrolytic cell which is divided into anode and cathode chambers with an ion exchange membrane and an aqueous solution of a trivalent chromium salt, such as chromium sulphate or chloride which is fed to the cathode chamber.

JP 61-288100 A describes a method for controlling pH in electrolytic treatment of steel sheets by monitoring the pH during the electrolytic treatment and liquid chemical dosing and calculating the required dose of the liquid chemical.

US 2005/0189231 A1 describes an electroplating bath for zinc-nickel ternary or higher alloys.

However there has been no success to date in developing a method by means of which the widespread hard-chrome plating from chromium(VI)-containing electrolytes was able to be replaced in commercial use. This can be attributed to the following points:
1. The chromium layers deposited from the previously known methods do not correspond to the requirements known for hard-chroming with respect to a layer thickness of 5 µm and above.
2. The hardness of the layers which can be deposited from these baths does not achieve the required layer hardnesses of at least 800 HV and above.
3. The known baths, with respect to reproducibility of the layers which can be deposited, do not deliver the qualities known from chromium(VI)-containing electrolytes. The chromium layers are very fissured from layer thicknesses of > 5 µm and detach from the underlying material.

These restrictions of the already known chroming electrolytes based on chromium(III) result from the rapidly changing pH value due to the reaction at the cathode and the oxidation of chromium(III) to chromium(VI) at the anode. Already known developments provide a separation of the anode and cathode space by a diaphragm or a cation exchanger membrane. The oxidation of chromium(III) ions at the anode is prevented by this membrane. The transport of the electrical current is ensured by H⁺ ions. This transport serves simultaneously for equalising the pH value which increases as a result of the hydrogen produced in the catholyte space.

Because of the jointly deposited chromium and the cationic salt radicals remaining in the catholyte, the result in the catholyte is a reduction in pH value which must be compensated for by the addition of a base, such as for example ammonia. The addition of ammonia leads as a rule to a locally greatly increasing pH value in the electrolyte, chromium hydroxide which is difficult to dissolve then being precipitated.

### SUMMARY OF THE INVENTION

Starting herefrom, it was the object of the present invention to provide a method with which reproducible deposition of chromium layers is made possible, which layers have a thickness which is sufficient for corrosion- or wear protection and have great hardness. The method is thereby intended to have a wide field of application and to be suitable in principle also for deposition of decorative layers.

This object is achieved by the method having the features of claim 1, the electroplating bath having the features of claim 8 and the hard-chrome surfaces having the features of claim 16. The further dependent claims reveal advantageous developments.

### DETAILED DESCRIPTION OF THE INVENTION

According to the invention, a method is provided for deposition of chromium layers with a thickness of at least 10 µm as hard-chrome plating for protection against wear or corrosion and/or as decorative chrome plating. The method is based on a part being connected as a cathode and being immersed in a catholyte comprising at least one chromium(III) salt and at least one compound stabilizing chromium(II) ions. An anolyte comprising a Brönsted acid is used at the same time. Catholyte and anolyte are separated by an anion-selective membrane, also termed anion exchanger membrane. In the present invention, it is in addition essential that at least one measuring device is used, by means of which deviations in pH value from a predefined pH value are monitored continuously. The predefined pH value is thereby determined as a function of the chromium(III) salts which are used so that an optimal chromium deposition is effected. In addition, a control device is used in the method according to the invention by means of which the pH value can be adjusted to the preset value in that automated addition of an acid or a base is effected.

The method according to the invention is characterised by the separation of the cathode and the anode space by an anion exchanger membrane. Mixing of the anolyte with the catholyte is prevented by the anion exchanger membrane. As a result, no chromium(III) ions pass to the anode side, as a result of which oxidation of chromium(III) ions into chromium(VI) ions at the anode can be prevented. By using the anode exchanger membranes, the chromium(III) ions which are present generally as cation complexes can likewise be prevented from penetrating through the membranes. The anolyte is contaminated with chromium ions during the coating not at all or only to a slight extent. The concentration of chromium(VI) ions in the anolyte can be prevented entirely by the addition of oxalic acid as reductive type to the anolyte. The addition of substances, such as ferrocyanides, to the anolyte or of sodium thiocyanates as described in GB 1 602 404, can be dispensed with entirely.

In the description of deposition mechanisms for the chromium deposition from chromium(III)-containing electrolytes into metallic chromium layers, it is assumed that the deposition extends further to metallic chromium via the steps chromium(III) to chromium(II). Since chromium(II) is oxidised very rapidly in air to form chromium(III), this cation must be stabilised. This can be effected preferably by the addition of amino acids or by urea. However it is also likewise possible to implement the electroplating under an inert gas atmosphere in order to prevent oxidation of the chromium(II).

Since during deposition of chromium layers the result is an increase in pH value as a result of hydrogen formation at the cathode and as a result of the transport of ions through the membrane, constant conditions during the chromium deposition can only be ensured by continuous monitoring of the electroplating bath with respect to the pH value. This is effected preferably by continuous circulation of the catholyte which flows through a pH measuring cell. If an increase in pH value results, acid can then be metered subsequently into the electrolyte by the control device.

A preferred variant thereby provides that the acid is removed from the anolyte in the continuous coating process and is subsequently metered into the catholyte. It is thereby likewise possible to add the acid to the catholyte via an external acid reservoir.

In addition, it is preferred that the temperature of the electroplating bath is also controlled in addition to the pH value. With the help of a temperature measuring cell, this is monitored and can then be adjusted to the desired value by means of a cooling or heating device.

A compound from the group consisting of ammonium chromium alum, potassium chromium alum, chromium chloride, chromium sulphate is selected preferably as chromium(III) salt or mixtures thereof are used. The concentration of chromium(III) salt is thereby preferably in a range of 0.1 mol/l up to the solubility limit of the salt or salt mixture in the catholyte.

There are used as compounds which stabilise chromium(II) ions amino acids, urea derivatives, aliphatic, mixed aromatic-aliphatic, cycloaliphatic or aromatic amines and/or amides. The concentration of these compounds is thereby preferably in the range of 0.5 mol/l to 3 mol/l, more preferably 0.5 mol/l to 1.2 mol/l relative to the catholyte.

According to the present invention, a buffer substance for buffering the pH value of the catholyte is added to the catholyte. This is selected thereby from the group consisting of the systems boric acid/borate, citric acid/citrate, aluminium³⁺/aluminium sulphate, oxalic acid/oxalate and/or tartaric acid/tartrate.

According to the present invention, wetting agents are added to the catholyte, which are selected from the group consisting of anionic and neutral surfactants, such as for example sodium lauryl sulphate, sodium dodecyl sulphate, polyethylene glycols, diisohexylsulphosuccinate, 2-ethylhexylsulphate, diisobutylsulphosuccinate, diisoamylsulphosuccinate and/or isodecylsulphosuccinate.

According to the invention, an electroplating bath is likewise provided for deposition of chromium layers with a thickness of at least 10 µm as hard-chrome plating for protection against wear or corrosion and/or as decorative chrome plating. The electroplating bath is based on a catholyte comprising at least one chromium(III) salt and at least one compound stabilizing chromium(II) ions selected from the group consisting of amino acids, urea, aliphatic, aromatic-aliphatic, cycloaliphatic or aromatic amines and/or amides, a buffer substance for buffering the pH value of the catholyte selected from the group consisting of the systems boric acid/borate, citric acid/citrate, aluminium³⁺/aluminium sulphate, oxalic acid/oxalate and/or tartaric acid/tartrate, and a wetting agent selected from the group consisting of anionic and/or neutral surfactants, and also an anolyte comprising a protonic acid. Catholyte and anolyte are hereby separated by an anion-selective membrane. In addition, the electroplating bath has a measuring device for continuous monitoring of deviations in pH value from a predefined pH value and also at least one control device for adjusting the pH value to the preset value. This is hereby effected by automated addition of an acid or a base. Advantageously, the anode is a dimensionally stable anode (DSA), i.e. an anode which does not dissolve under the operating conditions. As dimensionally stable anodes according to the invention there are thereby preferred anodes which comprise graphite or a lead alloy or titanium anodes which are coated with a mixed oxide and/or platinised. Coated or platinised anodes are thereby generally formed from titanium.

According to the invention, likewise hard-chrome surfaces are provided which can be produced according to the method according to the invention. These chromium layers have a thickness of at least 10 µm, the surface having a Vickers hardness according to EN ISO 6507 of at least 800 HV. According to the current density, high-gloss or also matt chromium layers can be deposited. The surfaces can of course serve also for decorative purposes.

### EXAMPLES

The subject according to the invention is intended to be explained in more detail with reference to the subsequent examples without wishing to restrict the latter to the special embodiments shown here.

### Comparative Example 1

A chromium layer deposited from a
Trichrome® electrolyte by the company Atotech.
According to the specifications of the manufacturer.
Bath temperature: 30°C
Current density: 8 A/dm²,
Deposition time: 25 minutes.
(see Fig. 1)

### Example 1

### Coating from ammonium chromium alum with glycin

### Composition of catholyte and anolyte

### Catholyte:

400 g/l ammonium chromium alum, the chromium content thereby corresponding to 10.6 per cent by mass.
40 g/l boric acid
80 g/l glycin
0.5 g/l sodium lauryl sulphate

### Anolyte:

30% H₂SO₄ dissolved in water

### Preparation of the catholyte:

Ammonium chromium alum (producible according to N. Rempfer, H-W Lerner, M. Bolte, Acta Cryst. (2004), E60, i80-i81) was heated for two hours with the addition of deionised water at 80°C. After cooling the ammonium chromium alum solution to 40°C, the boric acid and the glycin were added to the electrolyte. The pH value was subsequently adjusted to a pH value of 2.25 before the first coating by the addition of ammonia. The pH measuring device used was calibrated at 40°C.

The electroplating chromium deposition took place in a coating cell in which the anolyte (30% sulphuric acid) was separated from the catholyte (ammonium chromium alum batch) by an anion-exchanging membrane. The bath temperature during deposition was 40°C ± 2°C. The pH value chosen was between pH 2.2 and pH 2.3. During the test, platinised titanium was used as anode.

Cylindrical round bodies with a diameter of 1 cm and a length of 10 cm were coated. The test part was made of steel. Before the coating, the test part was cathodically degreased for 5 minutes at 60°C in an alkaline solution and subsequently for 30 seconds at a current density of 1 A/dm², rinsed in deionised water and pickled for 30 seconds in 5% sulphuric acid directly before the coating. During the coating, the cylindrical test part was rotated at 50^{1/min}.

15 A/dm² was set as cathodic current density. During the 2 hour coating, the pH value in the catholyte was maintained at 2.25 by metering anolyte thereto (see Fig. 2).
- **Result:**: Layer thickness 52.8 µm; measured with a light microscope (Zeiss - Axioplan) Hardness 833 HV measured on the microhardness tester (Anton Paar - MH-T4) Test load 50p, 10s, 5p/s (see Fig 3)

### Example 2

### Coating from ammonium chromium alum with diethanolamine

### Like example 1, diethanolamine was used instead of glycin

The batch of electrolyte and the sample pre-treatment corresponds to example 1. 1.1 mol/l diethanolamine is used instead of glycin as complex former.

The pH value was maintained at pH 2.3 to pH 2.5 during this test.
- Result:: Layer thickness 58.5 µm, measured with a light microscope (Zeiss-Axioplan) Hardness 855 HV measured on the microhardness tester (Anton Paar - MH-T4) Test load 50p, 10s, 5p/s

### Example 3

### Coating from chromium sulphate:

Test like example 1, instead of the ammonium chromium alum, chromium(3) sulphate with a concentration of 40 g Cr/l was used
- Result:: Layer thickness 39.8 µm; measured with a light microscope (Zeiss-Axioplan) Hardness 901 HV measured on the microhardness tester (Anton Paar - MH-T4) Test load 50p, 10s, 5p/s (see Fig. 5)

### Example 4

### Coating from chromium chloride:

### Catholyte:

1 mol/l chromium chloride
40 g/l aluminium sulphate
80 g/l glycin
0.5 g/l sodium lauryl sulphate

### Anolyte:

30% H₂SO₄ dissolved in water

The batch of electrolyte and the sample pre-treatment corresponds to the method according to claim 1. Aluminium sulphate instead of boric acid is used as buffer substance.

Sodium lauryl sulphate is added in addition as wetting agent to the catholyte.
- Result:: Layer thickness 10.8 µm; measured with a light microscope (Zeiss-Axioplan) Hardness 862 HV measured on the microhardness tester (Anton Paar - MH-T4) Test load 50p, 10s, 5p/s. (see Fig. 6)

### Example 5

### Coating from ammonium chromium alum with urea

### Like example 1, urea was used instead of glycin

The batch of electrolyte and the sample pre-treatment corresponds to example 1. 2 mol/l **urea** is used instead of glycin as complex former.

The pH value was maintained at pH 2.3 to pH 2.5 during this test.
- Result:: Layer thickness 28 µm, measured with a light microscope (Zeiss-Axioplan) Hardness 780 HV measured on the microhardness tester (Anton Paar - MH-T4) Test load 50p, 10s, 5p/s (s. Fig. 7)

### Example 6

### Coating from ammonium chromium alum with alanine

### Like example 1, alanine was used instead of glycin

The batch of electrolyte and the sample pre-treatment corresponds to example 1. 1 mol/l **alanine** is used instead of glycin as complex former.

The pH value was maintained at pH 2.3 to pH 2.5 during this test.
- Result:: Layer thickness 59.5 µm, measured with a light microscope (Zeiss-Axioplan) Hardness 760 HV measured on the microhardness tester (Anton Paar - MH-T4) Test load 50p, 10s, 5p/s (s. Fig. 8)

### BRIEF DESCRIPTION OF THE DRAWINGS

- Fig. 1:: Chromium layer from a conventional chromium(III) electrolyte
- Fig. 2:: Diagram of the test plant
- Fig. 3:: Sample from glycine bath
- Fig. 4:: Sample from diethanolamine electrolyte
- Fig. 5:: Sample from glycine chromium sulphate elec trolyte
- Fig. 6:: Sample from glycine chromium chloride electrolyte
- Fig. 7:: Sample from urea electrolyte
- Fig. 8:: Sample from alanine electrolyte

Fig. 2 shows a diagram of the inventive process. A power and control unit 1 monitors the following parameters of the electrolyte and controls the corresponding parts of the plant by sending control signals:
- Temperature of the electrolyte
- pH of the electrolyte
- recirculation of the electrolyte
- recirculation of the anolyte
- current for electroplating of the part being coated

By using a pump 2 for a base, a base selected from a liquid increasing the pH, e.g. ammonia, is added to the electrolyte in case of a decrease of the pH. This base is kept in a reservoir 3. The pump 2 receives the control signals from the power and control unit 1. By the use of a pump 4 for the acid, a liquid is added to the anolyte decreasing the pH. As a liquid for decreasing the pH, diluted sulphuric acid is preferred. The pump 4 receives the control signals from the power and control unit 1. The pH measuring device 5 amplifies signals from a pH probe in the measuring cell 6 and are relayed to the power and control unit 1. A pump 7 supplies the measuring cell 6 with fresh electrolyte which is taken from the reservoir 14. After finishing the measurement, the electrolyte is recirculated to the reservoir 14. The membrane anode 9 is an anode being encapsulated in an anion-exchanging membrane. The encapsulated anode is inside washed round by diluted sulphuric acid. The sulphuric acid is transported by an anolyte pump 10 from the reservoir 8 to the membrane anode 9. The sulphuric acid runs of by a second orifice of the membrane anode, which serves for the evacuation of the oxygen being generated at the anode. A further electrolyte pump 11 continuously transports electrolyte from the reservoir through a filter unit 12 and in circulation back to the reservoir 14. The part being coated in this process 13 is shown in the middle.

## Claims

1. Method for deposition of chromium layers with a thickness of at least 10 µm as hard-chrome plating for protection against wear or corrosion, in which a part is connected as a cathode and is immersed in a catholyte comprising at least one chromium(III) salt, at least one compound stabilizing chromium(II) ions selected from the group consisting of amino acids, urea, aliphatic, aromatic-aliphatic, cycloaliphatic or aromatic amines and/or amides, a buffer substance for buffering the pH value of the catholyte selected from the group consisting of the systems boric acid/borate, citric acid/citrate, aluminium³⁺/aluminium sulphate, oxalic acid/oxalate and/or tartaric acid/tartrate, a wetting agent selected from the group consisting of anionic and/or neutral surfactants,
and in which an anolyte comprising a Brönsted acid is used, wherein catholyte and anolyte being separated by an anion-selective membrane, and also, by means of at least one measuring device, deviations in the pH value from a predefined pH value are monitored continuously and, by means of at least one control device, the pH value is adjusted to the predefined value by automated addition of an acid or a base.

2. Method according to claim 1, wherein the acid is removed from the anolyte via the control device, said acid being metered subsequently into the catholyte in order to adjust the pH value.

3. Method according to one of the preceding claims, wherein the deviation in temperature of the electroplating bath from a predefined value is monitored continuously via a temperature measuring unit and the temperature of the electroplating bath is adjusted to the predefined value via a heating and/or cooling device.

4. Method according to one of the preceding claims, wherein the chromium(III) salt is selected from the group consisting of ammonium chromium alum, potassium chromium alum, chromium chloride, chromium sulphate and mixtures thereof, wherein the chromium(III) salt is preferably used in the catholyte in a concentration in the range of 0.1 mol/l up to the solubility limit of the salt.

5. Method according to one of the preceding claims, wherein the compound stabilizing chromium(II) ions is preferably used in the catholyte in a concentration of 0.5 mol/l to 3 mol/l, preferably 0.5 mol/l to 1.2 mol/l.

6. Method according to one of the preceding claims, wherein the wetting agent is selected from the group consisting of sodium lauryl sulphate, sodium dodecyl sulphate, polyethylene glycols, diisohexylsulphosuccinate, 2-ethylhexylsulphate, diisobutylsulphosuccinate, diisoamylsulphosuccinate and/or isodecylsulphosuccinate.

7. Method according to one of the preceding claims, wherein the anolyte contains sulphuric acid.

8. Electroplating bath for deposition of chromium layers with a thickness of at least 10 µm as hard-chrome plating for protection against wear or corrosion and/or as decorative chrome plating having a catholyte comprising at least one chromium(III) salt, at least one compound stabilizing chromium(II) ions selected from the group consisting of amino acids, urea, aliphatic, aromatic-aliphatic, cycloaliphatic or aromatic amines and/or amides, a buffer substance for buffering the pH value of the catholyte selected from the group consisting of the systems boric acid/borate, citric acid/citrate, aluminium³⁺/aluminium sulphate, oxalic acid/oxalate and/or tartaric acid/tartrate, and a wetting agent selected from the group consisting of anionic and/or neutral surfactants, and an anolyte comprising a protonic acid, catholyte and anolyte being separated by an anion-selective membrane, and also at least one measuring device for continuous monitoring of deviations in the pH value from a predefined pH value and at least one control device for adjusting the pH value to the preset value by automated addition of an acid or a base.

9. Electroplating bath according to claim 8,
wherein the control device for removing acid from the anolyte is in contact with the anolyte and, for metering of acid into the catholyte, is in contact with the catholyte.

10. Electroplating bath according to one of the claims 8 or 9, wherein the chromium(III) salt is selected from the group consisting of ammonium chromium alum, potassium chromium alum, chromium chloride, chromium sulphate and mixtures thereof.

11. Electroplating bath according to claim 10,
wherein the concentration of the at least one chromium(III) salt in the catholyte is preferably in the range of 0.1 mol up to the solubility limit of the salt.

12. Electroplating bath according to one of the claims 8 to 11, wherein the compound stabilizing chromium(II) ion is present in the catholyte in a concentration of 0.5 mol/l to 3 mol/l, preferably 0.5 mol/l to 1.2 mol/l.

13. Electroplating bath according to the preceding claim, wherein the wetting agent is selected from the group consisting of sodium lauryl sulphate, sodium dodecyl sulphate, polyethylene glycols, diisohexylsulphosuccinate, 2-ethylhexylsulphate, diisobutylsulphosuccinate, diisoamylsulphosuccinate and/or isodecylsulphosuccinate.

14. Electroplating bath according to one of the claims 8 to 13, wherein the anolyte contains sulphuric acid.

15. Electroplating bath according to one of the claims 8 to 14, wherein the electroplating bath has a dimensionally stable anode (DSA), which is preferably selected from the group consisting of graphite or anodes comprising a lead alloy, anodes coated with a mixed oxide and/or platinised anodes.

16. Hard-chrome surface which can be produced according to the method according to one of the claims 1 to 7, wherein the thickness of the chromium layer is at least 10 µm and the part surface having a Vickers hardness according to EN ISO 6507 of at least 800 HV.

## Patentansprüche

1. Verfahren zur Abscheidung von Chromschichten mit einer Dicke von mindestens 10 µm als Hartverchromung für den Verschleiß- oder Korrosionsschutz, bei dem ein Körper als Kathode geschaltet wird und in einen Katholyten eingetaucht wird, der mindestens ein Chrom(III)-Salz, mindestens eine Chrom(II)-Ionen stabilisierende Verbindung ausgewählt aus der Gruppe bestehend aus Aminosäuren, Harnstoff, aliphatischen, aromatisch-aliphatischen, cycloaliphatischen oder aromatischen Aminen und/oder Amiden, eine Puffersubstanz zur Pufferung des pH-Wertes ausgewählt aus der Gruppe bestehend aus den Systemen Borsäure/Borat, Citronensäure/Citrat Aluminium³+/Aluminiumsulfat und/oder Weinsäure/Tartrat, ein Netzmittel ausgewählt aus der Gruppe bestehend aus anionischen und/oder neutralen Tensiden enthält, und bei dem ein eine Brönsted-Säure enthaltender Anolyt eingesetzt wird, wobei Katholyt und Anolyt durch eine anionenselektive Membran getrennt werden, sowie mit mindestens einer Messvorrichtung Abweichungen des pH-Wertes von einem vordefinierten pH-Wert kontinuierlich überwacht werden und mit mindestens einer Regelungsvorrichtung der pH-Wert auf den vordefinierten Wert durch automatisierte Zugabe einer Säure oder einer Base eingestellt wird.

2. Verfahren nach Anspruch 1,
**dadurch gekennzeichnet, dass** über die Regelungsvorrichtung dem Anolyten Säure entnommen wird, die anschließend dem Katholyten zur Einstellung des pH-Wertes zudosiert wird.

3. Verfahren nach einem der vorhergehenden Ansprüche,
**dadurch gekennzeichnet, dass** über eine Temperatur-Messeinheit die Abweichung der Temperatur des Galvanisierungsbades von einem vordefinierten Wert kontinuierlich überwacht und über eine Heiz- und/oder Kühlvorrichtung die Temperatur des Galvanisierungsbades auf den vordefinierten Wert eingestellt wird.

4. Verfahren nach einem der vorhergehenden Ansprüche,
**dadurch gekennzeichnet, dass** das Chrom(III)-Salz ausgewählt ist aus der Gruppe bestehend aus Ammoniumchromalaun, Kaliumchromalaun, Chromchlorid, Chromsulfat und Mischungen hiervon, wobei das Chrom(III)-Salz bevorzugt in einer Konzentration im Bereich von 0,1 mol/l bis zur Löslichkeitsgrenze des Salzes im Katholyten eingesetzt wird.

5. Verfahren nach dem vorhergehenden Anspruch,
**dadurch gekennzeichnet, dass** die Chrom(II)-Ionen stabilisierende Verbindung in einer Konzentration von 0,5 mol/l bis 3 mol/l, bevorzugt von 0,5 mol/l bis 1,2 mol/l im Katholyten eingesetzt wird.

6. Verfahren nach dem vorhergehenden Anspruch,
**dadurch gekennzeichnet, dass** das Netzmittel ausgewählt ist aus der Gruppe bestehend aus Natriumlaurylsulfat, Natriumdodecylsulfat, Polyethylenglykolen, Diisohexylsulfosuccinat, 2-Ethylhexylsulfat, Diisobutylsulfosuccinat, Diisoamylsulfosuccinat und/oder Isodecylsulfosuccinat.

7. Verfahren nach einem der vorhergehenden Ansprüche,
**dadurch gekennzeichnet, dass** der Anolyt Schwefelsäure enthält.

8. Galvanisierungsbad zur Abscheidung von Chromschichten mit einer Dicke von mindestens 10 µm als Hartverchromung für den Verschleiß- oder Korrosionsschutz und/oder als dekorative Verchromung mit einem Katholyten, der der mindestens ein Chrom(III)-Salz, mindestens eine Chrom(II)-Ionen stabilisierende Verbindung ausgewählt aus der Gruppe bestehend aus Aminosäuren, Harnstoff, aliphatischen, aromatisch-aliphatischen, cycloaliphatischen oder aromatischen Aminen und/oder Amiden, eine Puffersubstanz zur Pufferung des pH-Wertes ausgewählt aus der Gruppe bestehend aus den Systemen Borsäure/Borat, Citronensäure/Citrat Aluminium³⁺/Aluminiumsulfat und/oder Weinsäure/Tartrat, ein Netzmittel ausgewählt aus der Gruppe bestehend aus anionischen und/oder neutralen Tensiden enthält, und einem eine Protonensäure enthaltenden Anolyten, wobei Katholyt und Anolyt durch eine anionenselektive Membran getrennt sind, sowie mindestens einer Messvorrichtung zur kontinuierlichen Überwachung von Abweichungen des pH-Wertes von einem vordefinierten pH-Wert und mindestens einer Regelungsvorrichtung zur Einstellung des pH-Wertes auf den vorjustierten Wert durch automatisierte Zugabe einer Säure oder einer Base.

9. Galvanisierungsbad nach Anspruch 8,
**dadurch gekennzeichnet, dass** die Regelungsvorrichtung zur Entnahme von Säure aus dem Anolyten in Kontakt mit dem Anolyten und zur Zudosierung von Säure zu dem Katholyten in Kontakt mit dem Katholyten steht.

10. Galvanisierungsbad nach einem der Ansprüche 8 oder 9,
**dadurch gekennzeichnet, dass** das Chrom(III)-Salz ausgewählt ist aus der Gruppe bestehend aus Ammoniumchromalaun, Kaliumchromalaun, Chromchlorid, Chromsulfat und Mischungen hiervon.

11. Galvanisierungsbad nach Anspruch 10,
**dadurch gekennzeichnet, dass** die Konzentration des mindestens einen Chrom(III)-Salzes im Bereich von 0,1 mol/l bis zur Löslichkeitsgrenze des Salzes im Katholyten liegt.

12. Galvanisierungsbad nach einem der Ansprüche 8 bis 11,
**dadurch gekennzeichnet, dass** die Chrom(II)-Ionen stabilisierende Verbindung in einer Konzentration von 0,5 mol/l bis 3 mol/l, bevorzugt von 0,5 mol/l bis 1,2 mol/l im Katholyten vorliegt.

13. Galvanisierungsbad nach dem vorhergehenden Anspruch,
**dadurch gekennzeichnet, dass** das Netzmittel ausgewählt ist aus der Gruppe bestehend aus Natriumlaurylsulfat, Natriumdodecylsulfat, Polyethylenglykolen, Diisohexylsulfosuccinat, 2-Ethylhexylsulfat, Diisobutylsulfosuccinat, Düsoamylsulfosuccinat und/oder Isodecylsulfosuccinat.

14. Galvanisierungsbad nach einem der Ansprüche 8 bis 13,
**dadurch gekennzeichnet, dass** der Anolyt Schwefelsäure enthält.

15. Galvanisierungsbad nach einem der Ansprüche 8 bis 14,
**dadurch gekennzeichnet, dass** das Galvanisierungsbad eine dimensionsstabile Anode (DSA) aufweist, die bevorzugt ausgewählt ist aus der Gruppe bestehend aus Graphit oder einer Bleilegierung enthaltenden Anoden, mit einem Mischoxid beschichteten Anoden und/oder platinierten Anoden.

16. Hartverchromte Oberfläche, die nach dem Verfahren nach einem der Ansprüche 1 bis 7 herstellbar ist, wobei die Dicke der Chromschicht mindestens 10 µm beträgt und die Körperoberfläche eine Vickers-Härte nach EN ISO 6507 von mindestens 800 HV aufweist.

## Revendications

1. Procédé de dépôt de couches de chrome avec une épaisseur d'au moins 10 µm sous forme d'un chromage dur pour la protection contre l'usure ou la corrosion, dans lequel une pièce est reliée en tant que cathode et est plongée dans un catholyte comprenant au moins un sel de chrome (III), au moins un composé de stabilisation des ions chrome (II) choisi dans le groupe consistant en acides aminés, urée, amines et/ou amides aliphatiques, aromatiques-aliphatiques, cycloaliphatiques ou aromatiques, une substance tampon pour tamponner la valeur de pH du catholyte choisie dans le groupe consistant en systèmes acide borique/borate, acide citrique/citrate, aluminium³⁺/sulfate d'aluminium, acide oxalique/oxalate et/ou acide tartrique/tartrate, un agent mouillant choisi dans le groupe consistant en tensioactifs anioniques et/ou neutres,
et dans lequel un anolyte comprenant un acide de Brönsted est utilisé, catholyte et anolyte étant séparés par une membrane sélective vis-à-vis des anions, et également, au moyen d'au moins un dispositif de mesure, des écarts de valeur de pH par rapport à une valeur de pH prédéfinie sont surveillés de manière continue et, au moyen d'au moins un dispositif de commande, la valeur de pH est ajustée à la valeur prédéfinie par l'addition automatisée d'un acide ou d'une base.

2. Procédé selon la revendication 1, dans lequel l'acide est éliminé de l'anolyte par le dispositif de commande, ledit acide étant mesuré ultérieurement dans le catholyte afin d'ajuster la valeur de pH.

3. Procédé selon l'une des revendications précédentes, dans lequel l'écart de température du bain galvanoplastique à partir d'une valeur prédéfinie est surveillé de manière continue par une unité de mesure de la température et la température du bain galvanoplastique est ajustée à la valeur prédéfinie par un dispositif de chauffage et/ou refroidissement.

4. Procédé selon l'une des revendications précédentes, dans lequel le sel de chrome (III) est choisi dans le groupe consistant en alun d'ammonium et de chrome, alun de potassium et de chrome, chlorure de chrome, sulfate de chrome et des mélanges de ces derniers, dans lequel le sel de chrome (III) est utilisé de préférence dans le catholyte à une concentration dans le domaine allant de 0,1 mol/l jusqu'à la limite de solubilité du sel.

5. Procédé selon l'une des revendications précédentes, dans lequel le composé de stabilisation des ions chrome (II) est utilisé de préférence dans le catholyte à une concentration de 0,5 mol/l à 3 mol/l, de préférence de 0,5 mol/l à 1,2 mol/l.

6. Procédé selon l'une des revendications précédentes, dans lequel l'agent mouillant est choisi dans le groupe consistant en laurylsulfate de sodium, dodécylsulfate de sodium, polyéthylène glycols, diisohexylsulfosuccinate, 2-éthylhexylsulfate, diisobutylsulfosuccinate, diisoamylsulfosuccinate et/ou isodécylsulfosuccinate.

7. Procédé selon l'une des revendications précédentes, dans lequel l'anolyte contient de l'acide sulfurique.

8. Bain galvanoplastique pour le dépôt de couches de chrome avec une épaisseur d'au moins 10 µm sous forme d'un chromage dur pour la protection contre l'usure ou la corrosion et/ou sous forme d'un chromage décoratif ayant un catholyte comprenant au moins un sel de chrome (III), au moins un composé de stabilisation des ions chrome (II) choisi dans le groupe consistant en acides aminés, urée, amines et/ou amides aliphatiques, aromatiques-aliphatiques, cycloaliphatiques ou aromatiques, une substance tampon pour tamponner la valeur de pH du catholyte choisie dans le groupe consistant en systèmes acide borique/borate, acide citrique/citrate, aluminium³⁺/sulfate d'aluminium, acide oxalique/oxalate et/ou acide tartrique/tartrate, et un agent mouillant choisi dans le groupe consistant en tensioactifs anioniques et/ou neutres, et un anolyte comprenant un acide protonique, catholyte et anolyte étant séparés par une membrane sélective vis-à-vis des anions, et également, au moins un dispositif de mesure pour la surveillance continue des écarts de la valeur de pH à partir d'une valeur de pH prédéfinie et au moins un dispositif de commande pour ajuster la valeur de pH à la valeur prédéfinie par l'addition automatisée d'un acide ou d'une base.

9. Bain galvanoplastique selon la revendication 8, dans lequel le dispositif de commande pour éliminer l'acide de l'anolyte est en contact avec l'anolyte et, pour mesurer l'acide dans le catholyte, est en contact avec le catholyte.

10. Bain galvanoplastique selon l'une des revendications 8 ou 9, dans lequel le sel de chrome (III) est choisi dans le groupe consistant en alun d'ammonium et de chrome, alun de potassium et de chrome, chlorure de chrome, sulfate de chrome et des mélanges de ces derniers.

11. Bain galvanoplastique selon la revendication 10, dans lequel la concentration du au moins un sel de chrome (III) dans le catholyte se situe de préférence dans le domaine allant de 0,1 mole jusqu'à la limite de solubilité du sel.

12. Bain galvanoplastique selon l'une des revendications 8 à 11, dans lequel le composé stabilisant l'ion chrome (II) est présent dans le catholyte à une concentration de 0,5 mol/l à 3 mol/l, de préférence de 0,5 mol/l à 1,2 mol/l.

13. Bain galvanoplastique selon la revendication précédente, dans lequel l'agent mouillant est choisi dans le groupe consistant en laurylsulfate de sodium, dodécylsulfate de sodium, polyéthylène glycols, diisohexylsulfosuccinate, 2-éthylhexylsulfate, diisobutylsulfosuccinate, diisoamylsulfosuccinate et/ou isodécylsulfosuccinate.

14. Bain galvanoplastique selon l'une des revendications 8 à 13, dans lequel l'anolyte contient de l'acide sulfurique.

15. Bain galvanoplastique selon l'une des revendications 8 à 14, lequel bain galvanoplastique possède une anode dimensionnellement stable (DSA), qui est choisie de préférence dans le groupe consistant en graphite ou anodes comprenant un alliage de plomb, des anodes revêtues d'un oxyde mixte et/ou des anodes platinées.

16. Surface au chromage dur qui peut être produite selon le procédé selon l'une des revendications 1 à 7, dans laquelle l'épaisseur de la couche de chrome est d'au moins 10 µm et la surface de la pièce ayant une dureté Vickers selon la norme EN ISO 6507 d'au moins 800 HV.
